

## 1

3,220,948

## LUBRICATING OIL ADDITIVES

Johannes Reese, Wiesbaden, and Berthold Brähler, Fulda, Germany, assignors to Chemische Werke Albert, Wiesbaden-Biebrich, Germany, a corporation of Germany  
No Drawing. Filed Mar. 20, 1962, Ser. No. 181,172  
Claims priority, application Germany, Mar. 24, 1961,  
C 23,726

16 Claims. (Cl. 252—46.6)

The invention relates to novel lubricating additives for improving the properties of lubricating oils. The invention also relates to improved lubricating oils containing the novel lubricating additives.

It is well known that lubricating oils such as refined mineral oils do not meet the standards required for their use as engine oils or transmission lubricants. Attempts to overcome the disadvantages of oils such as those prepared by petroleum distillation or by the Fischer-Tropsch synthesis have led to the use of different types of additives. The resulting oils are called alloyed oils.

One of the principal defects of the basic oils is their inadequate temperature-viscosity index. Another defect is their loss of uniform films on metal surfaces when under pressure. For example, at points of transmission of heavy weights such as when gear wheels pass over a transmission gear the oil films frequently break so that the conditions and wear values are almost that of dry operation.

The transmission and engine oils also require anti-corrosive properties to prevent the corrosion of the lubricated parts and the oil itself. The corrosion by oil and the aging of the oil, i.e., the degradation of the oil is catalytically favored particularly in the presence of oxygen, by metallic particles, formed by abrasion. Therefore, in order to be satisfactory, the additives must act as inhibitors.

Two very important effects which are obtained by the addition of additives to the oil are the "detergent effect" and the "dispersant effect." These additives are usually referred to as HD or DD additives which are abbreviations for "heavy duty" or "detergent-dispersant" additives. These additives clean the lubricated parts by automatically removing metallic residues and carbonization residues from the lubricated surfaces and dispersing the said residues in the oil.

All of the afore-said problems involve surface tension problems and therefore it is not surprising that most oil additives have surface active properties, are similar in principle, and their ranges of activity frequently overlap. The additives have a strongly polar portion and an oleophilic portion in their molecules. The surface active additives form a sort of adhesive bridge between the metal and the oil since the oleophilic portion of the molecule projects into the oil while the polar portion of the molecule covers the metal surface. This gives a better mechanic capacitance to the oil film.

Many compounds ranging from simple metal soaps to complex sulfur-phosphorus compounds have been proposed as lubricating oil additives. Many patents describe the reflux reaction products of partly oxygen-free, partly oxygen-containing low molecular weight or high molecular weight organic compounds with phosphorus-sulfides which may subsequently be treated with metal oxides, such as the oxides of barium, calcium or zinc. Special attention has been given to dithiophosphoric acid esters and their salts which are prepared by the reaction of high molecular weight alcohols with phosphorus-penta-sulfide followed by neutralization of the acid esters with a metal oxide to form salts such as Zn-O,O-dihexyldithiophosphate. It has also been proposed to use mixtures of derivatives of dithiophosphoric acid and organic poly-

## 2

sulfides. In German Auslegeschrift No. 1,042,807 there are described lubricating oil additives consisting of mixtures of a phosphoric compound selected from the group consisting of (A) an oil soluble dithiophosphoric acid triester, a metal salt of dithiophosphoric acid diesters, a bis-(dithiophosphoric acid diester) or a dithiophosphoric acid diester-thioanhydride and (B) an oil soluble turpentine-polysulfide or an oil soluble di-,aralkyl polysulfide. However, satisfying results are obtained only by using critical amounts of the two components. Recently efforts have been made to obtain ash-free additives which have not been available.

It is an object of the invention to provide novel lubricating additives for improving the dispersent-detergent properties of lubricating oils.

It is another object of the invention to provide improved lubricating oils containing novel lubricating additives.

These and other objects and advantages of the invention will become obvious from the following detailed description.

The lubricating additives of the invention are compatible in all proportions with the lubricating oils and consist of a combination product, i.e., a mixture or a reaction product, of (A) 10 to 90% by weight of one or more O,O-diesters of dithiophosphoric acid and a monohydric aliphatic alcohol which esters are already known as lubricating additives, and (B) 90 to 10% by weight of the reaction product of sulfur and a diester of an  $\alpha,\beta$ -unsaturated dicarboxylic acid and a monohydric aliphatic alcohol. As the term "aliphatic" indicates, the characteristic feature of these radicals is their non-aromatic structure, and therefore the term "aliphatic" is generic for cycloaliphatic, too. The monohydric aliphatic alcohols consist of an OH-group and hydrocarbon radicals having 4 to 22 carbon atoms. The reaction product of sulfur and said diester is hereinafter referred to as "sulfurized ester". Preferably the mixtures contain 30 to 70% by weight of the said dithiophosphoric acid ester and 70 to 40% by weight of the said reaction product.

Examples of suitable  $\alpha,\beta$ -unsaturated dicarboxylic acids whose esters may be used are itaconic acid, mesaconic acid, citraconic acid, maleic acid and fumaric acid. Maleic acid and fumaric acid are the preferred acids.

The alcohols from which the alkyl portion of the esters are derived are branched or straight chain aliphatic or cycloaliphatic hydrocarbon alcohols which have 4 to 22 carbon atoms. Examples of suitable alcohols are butyl alcohol, isobutyl alcohol, cyclohexanol, 2-ethylhexanol, n-octanol, diisobutanol, dodecyl alcohol alcohol, oleyl alcohol, stearyl alcohol, commercial mixtures of fatty alcohols, i.e. those obtained by a hydrolysis of fats or fatty oils of natural origin such as coconut oil or lard or of ester waxes and subsequent hydrogenation, e.g., alcohols having 12 to 18 carbon atoms, etc.

The components can be mixed at temperatures ranging from room temperature to 200° C., preferably between room temperature and 120° C. If the components are mixed at temperatures higher than room temperature, a reaction takes place. If the mixing is carried out at a relatively low temperature such as room temperature, the mixture may be subsequently heated to a higher temperature to cause a reaction.

The lubricating oils to which the additives of the invention are added are animal, vegetable, mineral or synthetic oils. It is preferred, however, to use oils obtained in the petroleum industry. The improved lubricating oils contain 0.2 to 10%, preferably 0.5 to 3%, by weight of the additive mixture calculated on the basis of the weight of the lubricating oil. The lubricating oil products have properties satisfactory for "HD" and "EP" oils and may

be used for various purposes such as breaking-in oils for engines or hypoid gear oils. Other known lubricating additives may be added to the improved lubricating oils such as additives for improving the temperature-viscosity index.

The O,O-dialkylthiophosphoric acid esters are known compounds and can be prepared by known means. For example, the alcohol to be reacted is dissolved in an inert organic solvent and while maintaining the mixture at a slightly elevated temperature, the phosphorus pentasulfide

beölen," Erdöl und Kohle, vol. 7 (1954), p. 640-42, was carried out.

#### IFE test

A basic oil of the Deutsche Gasolin-Nitag type (Type SAE 90,  $d_2^{20}=0.918$ ) was used for the tests. The additives to be tested were added to the basic oil so that the basic oil contained 2% by weight of the additives. The results of the tests are summarized in Table I.

TABLE I

| Additive                                 | Type of testing                                                  | Wear value<br>in grams<br>$\times 10^{-4}$ | Initial and end tem-<br>perature, ° C. |                        | Sliding trace On the surface                                                                                                        |
|------------------------------------------|------------------------------------------------------------------|--------------------------------------------|----------------------------------------|------------------------|-------------------------------------------------------------------------------------------------------------------------------------|
|                                          |                                                                  |                                            | With oil<br>Feeding                    | Without oil<br>Feeding |                                                                                                                                     |
| None                                     | Normal                                                           | 33.20<br>0.80<br>4.82                      | 94/116                                 | -----                  | Many thin grooves, dark gray.                                                                                                       |
|                                          | Normal                                                           |                                            | 92/118                                 | -----                  | Smooth, slightly violet.                                                                                                            |
|                                          | High speed                                                       |                                            | 176/204                                | -----                  | Smooth, violet with light yellow foundation (tarnishing color of the steel), dark blue tarnishing color besides the sliding traces. |
| O,O-dialkyl-dithiophosphoric acid ester. | Emergency test without oil<br>(after 19 minutes and 30 seconds). | 2.20                                       | 97/120                                 | 120/166                | Isolated thin grooves, foundation of the grooves a dark gray.                                                                       |
|                                          | Normal                                                           |                                            | 92/113                                 | -----                  | Finest grooves, dark brown with a violet sheen.                                                                                     |
|                                          | (Normal)                                                         |                                            | 81/81                                  | -----                  | Apart from some isolated finest grooves, smooth, violet, good cooling activity, separation on the sliding trace.                    |
| Sulphurized fumaric acid dibutyl ester.  | High speed                                                       | 3.01<br>0.98<br>0.58                       | 73/71                                  | -----                  | Smooth, violet.                                                                                                                     |
|                                          | Normal                                                           |                                            | -----                                  | -----                  | -----                                                                                                                               |
|                                          | Emergency test without oil<br>(after 43 minutes).                |                                            | 89/113                                 | 86/147                 | -----                                                                                                                               |
| Additive of Example I                    |                                                                  |                                            |                                        |                        |                                                                                                                                     |

Normal-test: 3 hours at 150 r.p.m.,\* sliding speed 0.2 m/second, bearing pressure 4,500 kg./cm.<sup>2</sup>.

High speed: 1 hour at 450 r.p.m.,\* sliding speed 0.6 m/second, bearing pressure 4,500 kg./cm.<sup>2</sup>.

Emergency test without oil: 3 hours normal test, then oil feeding was stopped, at the moment that the piston started to seize the apparatus was stopped (indication of the time and of the wear value at this moment).

\*R.p.m.=revolutions per minute.

is gradually added until the reaction is completed. After filtration and elimination of the solvent, the product can be purified by distillation or crystallization of its salts although purification is not required.

The sulfurized ester of the  $\alpha,\beta$ -unsaturated carboxylic acids may be prepared by a process similar to that described by Michael, Berichte der Deutschen Chem. Gesellschaft, vol. 28 (1895), p. 1633, or by Flett et al., Maleic Anhydride Derivatives (1952), p. 219. Thus, for example, one mol of diethyl fumarate is heated with one gramatom or an excess of sulfur at an elevated temperature until completion of the reaction; the mixture is then cooled and the unreacted ester and sulfur are separated from the product. Michael refers to his reaction product as episulfidiosuccinic acid diethylester but we believe the product to be a dimer, possibly 1,4-dithia-cyclohexane-2,3,4,5-tetracarboxylic acid tetraethyl ester, because of its molecular weight determination and its behavior during the reaction.

In the following examples there are described several preferred embodiments to illustrate the invention. However, it should be understood that the invention is not intended to be limited to the specific embodiment.

35 40 45 50 55

#### FZG—gear wheel—short test

This test was conducted with the same basic oil as the IFE test containing 2% by weight of the additive of Example I. Also tested were the basic oil and a standard alloyed oil now sold commercially. The rotary speed ( $v$ ) was 8.3 m./second at 2,175 r.p.m. with the initial temperature of the oil container at 90° C. The sliding speed on the tooth crest ( $V_g$ ) was 0.675  $v$  m./second. The basic oil failed at a load range of 7 and the commercial alloyed oil failed at a load range of 10. In contrast thereto, the basic oil containing the additive of Example I had a load range of above 12, the maximum obtainable. This means that no gear damage had been encountered in the highest load range by a specific wear  $V_s$  below 0.1 mg. per HP.h. (horse power hour).

The above tests clearly show the advantages of the additives of the invention. It is surprising to note that neither the sulfurized fumaric acid ester nor the dithiophosphoric acid ester alone yield satisfactory results, while the reaction product gives satisfactory results. These superior results are clearly shown by the high speed test and the emergency test without oil.

#### EXAMPLE II

121 parts by weight of dithiophosphoric acid-O,O-di(isobutyl) ester were mixed with 130 parts by weight of a sulfurized product of di-isobutyl fumarate and the mixture was heated for 6 hours at 120° C. A dark brown oil of  $n_D^{20}=1.4860$  was obtained which could be mixed with lubricating oils in any desired proportion. The IFE test of this product showed that it was a suitable additive for preparing breaking-in engine oils.

60 65 70 75

#### EXAMPLE III

151 parts by weight of a dithiophosphoric acid-O,O-di-alkylester were mixed with 60 parts by weight of a sulfurized dialkyl fumarate at room temperature and a medium brown, clear oily product was obtained which was compatible with lubricating oils in any proportion. The alkyl radicals of the said esters were derived from a mixture of fatty alcohols having 12 to 18 carbon atoms. When the

#### EXAMPLE I

251 parts by weight of an O,O-dialkyl-dithiophosphoric acid ester wherein the alkyl radicals are derived from a commercial mixture of fatty alcohols having 12 to 18 carbon atoms and which has an acid number of 100 were heated with 130 parts by weight of a sulfurized dibutyl fumarate reaction product for 12 hours at 120° C., 370 parts of a dark brown, clear oil of  $n_D^{20}=1.4780$  were obtained. The product was compatible in all proportions with lubricating oils.

To illustrate the superior efficiency of the additives of the invention the IFE test described by Bartel et al., "Untersuchungen über Verschleiss und Reibung," Schmiertechnik, vol 3, issue 4 (1956), p 184-191 and FZG-gear wheel-short test of Niemann et al., "Erfahrungen mit der Getriebeölprüfung im Zahnradverspannungsprüfstand," Erdöl und Kohle, vol. 12 (1959), p. 472-80, and "Der FZG-Zahnrad-Kurztest zur Prüfung von Getrie-

product was added to a basic oil in an amount of 5% by weight, a gear oil of good quality was obtained.

## EXAMPLE IV

151 parts by weight of a dithiophosphoric acid-O,O-di-alkylester wherein the alkyl radicals were derived from fatty alcohols having 12 to 18 carbon atoms was mixed with 112 parts by weight of a sulfurized di-(2-ethylhexyl) fumarate for 25 hours at 120° C. A brown oil of

$$n_{D}^{20} = 1.4776$$

was obtained. The said oil was compatible in any desired proportion with lubricating oils and was a suitable additive for gear oils.

## EXAMPLE V

30 parts by weight of dithiophosphoric acid-O,O-di-butylester was mixed at room temperature with 130 parts by weight of a sulfurized dibutyl fumarate. The resulting composition was a suitable additive for the preparation of breaking-in engine oils.

Various modifications of the products of the invention may be made without departing from the spirit or scope thereof, and it is to be understood that the invention is to be limited only as defined in the appended claims.

We claim:

1. A lubricating oil additive consisting of a reaction product formed by heating up to 200° C. a mixture of (A) 10 to 90% by weight of a dithiophosphoric acid-O,O-di-alkyl ester and (B) 90 to 10% by weight of the reaction product of sulfur and a dialiphatic ester of an  $\alpha,\beta$ -ethylenically unsaturated dicarboxylic acid wherein the aliphatic radicals are hydrocarbon radicals having 4 to 22 carbon atoms.

2. The additive of claim 1 wherein the  $\alpha,\beta$ -unsaturated dicarboxylic acid is selected from the group consisting of maleic acid and fumaric acid.

3. A lubricating oil additive consisting of a reaction product formed by heating up to 200° C. a mixture of (A) 30 to 70% by weight of a dithiophosphoric acid-O,O-di-alkyl ester and (B) 70 to 30% by weight of the reaction product of sulfur and a dialiphatic ester of an  $\alpha,\beta$ -ethylenically unsaturated dicarboxylic acid wherein the aliphatic radicals are hydrocarbon radicals having 4 to 22 carbon atoms.

4. A lubricating oil additive consisting of a reaction product formed by heating up to 200° C. a mixture of (A) 30 to 70% by weight of a dithiophosphoric acid-O,O-di-alkylester wherein the alkyl radicals are derived from a mixture of fatty alcohols having 12 to 18 carbon atoms and (B) 70 to 30% by weight of a sulfurized product of dibutyl fumarate.

5. A lubricating oil additive consisting of a reaction product formed by heating up to 200° C. a mixture of 30 to 70% by weight of a dithiophosphoric acid-O,O-di-(isobutyl)-ester and (B) 70 to 30% by weight of a sulfurized product of di-(isobutyl) fumarate.

6. A lubricating oil additive consisting of a reaction product formed by heating up to 200 C. a mixture of (A) 30 to 70% by weight of a dithiophosphoric acid-O,O-di-alkylester and (B) 70 to 30% by weight of a sulfurized product of dialkyl fumarate wherein the alkyl radical of the esters are derived from a mixture of fatty alcohols having 12 to 18 carbon atoms.

7. A lubricating oil additive consisting of a reaction product formed by heating up to 200° C. a mixture of (A) 30 to 70% by weight of a dithiophosphoric acid-O,O-di-alkylester wherein the alkyl radicals are derived from a mixture of fatty alcohols having 12 to 18 carbon atoms and (B) 70 to 30% by weight of a sulfurized product of di-(2-ethylhexyl) fumarate.

8. A lubricating oil additive consisting of a reaction product formed by heating up to 200° C. a mixture of (A) 30 to 70% by weight of dithiophosphoric acid-O,O-di-

butylester and (B) 70 to 30% by weight of a sulfurized product of dibutyl fumarate.

9. An improved lubricating oil comprising a major amount of an oil suitable as a base in lubricating oils and containing 0.2 to 10% calculated on the weight of the oil, of a lubricating oil additive consisting of a reaction product formed by heating up to 200° C. a mixture of (A) 10 to 90% by weight of a dithiophosphoric acid-O,O-di-alkyl ester and (B) 90 to 10% by weight of the reaction product of sulfur and a dialiphatic ester of an  $\alpha,\beta$ -ethylenically unsaturated dicarboxylic acid wherein the aliphatic radicals are hydrocarbon radicals having 4 to 22 carbon atoms.

10. The lubricating oil of claim 9 wherein the amount of lubricating oil additive is 0.5 to 3% by weight.

11. The lubricating oil of claim 9 wherein the  $\alpha,\beta$ -ethylenically unsaturated dicarboxylic acid is selected from the group consisting of maleic acid and fumaric acid.

12. An improved lubricating oil comprising a major amount of an oil suitable as a base in lubricating oils and containing 0.2 to 10%, calculated on the weight of the oil, of a lubricating oil additive consisting of a reaction product formed by heating up to 200° C. a mixture of (A) 30 to 70% by weight of a dithiophosphoric acid-O,O-di-alkylester wherein the alkyl radicals are derived from a mixture of fatty alcohols having 12 to 18 carbon atoms and (B) 70 to 30% by weight of a sulfurized product of dibutyl fumarate.

13. An improved lubricating oil comprising a major amount of an oil suitable as a base in lubricating oils and containing 0.2 to 10%, calculated on the weight of the oil, of a lubricating oil additive consisting of a reaction product formed by heating up to 200° C. a mixture of (A) 30 to 70% by weight of a dithiophosphoric acid-O,O-di-(isobutyl)-ester and (B) 70 to 30% by weight of a sulfurized product of di-(isobutyl) fumarate.

14. An improved lubricating oil comprising a major amount of an oil suitable as a base in lubricating oils and containing 0.2 to 10%, calculated on the weight of the oil, of a lubricating oil additive consisting of a reaction product formed by heating up to 200° C. a mixture of (A) 30 to 70% by weight of a dithiophosphoric acid-O,O-di-alkylester and (B) 70 to 30% by weight of a sulfurized product of dialkyl fumarate wherein the alkyl radicals of the esters are derived from a mixture of fatty alcohols having 12 to 18 carbon atoms.

15. An improved lubricating oil comprising a major amount of an oil suitable as a base in lubricating oils and containing 0.2 to 10%, calculated on the weight of the oil, of a lubricating oil additive consisting of a reaction product formed by heating up to 200° C. a mixture of (A) 30 to 70% by weight of a dithiophosphoric acid-O,O-di-alkylester wherein the alkyl radicals are derived from a mixture of fatty alcohols having 12 to 18 carbon atoms and (B) 70 to 30% by weight of a sulfurized product of di-(2-ethylhexyl) fumarate.

16. An improved lubricating oil comprising a major amount of an oil suitable as a base in lubricating oils and containing 0.2 to 10%, calculated on the weight of the oil, of a lubricating oil additive consisting of a reaction product formed by heating up to 200° C. a mixture of (A) 30 to 70% by weight of dithiophosphoric acid-O,O-di-butylester and (B) 70 to 30% by weight of a sulfurized product of dibutyl fumarate.

## References Cited by the Examiner

## UNITED STATES PATENTS

|           |         |           |            |
|-----------|---------|-----------|------------|
| 2,220,843 | 11/1940 | Johnson   | 252—48.6 X |
| 2,242,260 | 5/1941  | Prutton   | 292—46.6   |
| 2,773,861 | 12/1956 | Musselman | 252—46.6 X |
| 2,827,434 | 3/1958  | Wierber   | 252—48.6 X |

DANIEL E. WYMAN, Primary Examiner.

ALPHONSO D. SULLIVAN, Examiner.